

## UNITED STATES PATENT OFFICE

2,214,059

## DIESEL FUEL

Eugene Lieber, Linden, N. J., and Pharis Miller,  
Des Moines, Iowa, assignors to Standard Oil  
Development Company, a corporation of Dela-  
ware

No Drawing. Application July 14, 1938,  
Serial No. 219,158

3 Claims. (Cl. 44—9)

This invention relates to improved Diesel fuels and methods for preparing the same. More particularly, this invention relates to the incorporation of a novel type of ignition-promoting agent into a hydrocarbon Diesel fuel stock, such as a gas oil fraction of petroleum origin; this novel type of agent being a compound containing an active linkage in an oxy-nitrogen sulfur group attached to carbon, such as a nitrosyl mercaptan, and possessing suitable solubility in the oil, resistance to hydrolysis, and properties for conferring on the fuel undergoing combustion in a compression-ignition engine excellent ignition qualities. 10 In consideration of increasing the power, fuel economy, and the reduction of vibration in the operation of compression-ignition engines when the hydrocarbon fuel contains insufficient amounts of the compounds recognizable as serving these ends, the additions of various non-hydrocarbon compounds, often spoken of as dopes, such as certain nitroso compounds and alkyl polysulfides have been proposed. Some of these dopes have been represented as being explosive 20 primers for initiating the ignition at low temperatures.

In many instances the addition agents or dopes proposed by the prior art have been difficult to use. Some are too volatile and therefore reduce the flash point of the doped fuel to below a safe temperature. Some must be added in large amounts to be effective and in such amounts may produce undesirable amounts of corrosive combustion products. Some are unstable when exposed to moisture, and some are too explosive. 30

Ignition qualities of a compression-ignition fuel are promoted not only by an easy starting of the ignition but also by other factors comprising combustion with regulated rapidity to avoid too abrupt accumulation of pressure which causes detonation. 40

A prime consideration in the use of addition agents or dopes for Diesel fuels, aside from their beneficial effects on the ignition qualities of the fuel and detrimental effects, is the cost. It can be readily seen that substances which can be manufactured by simple reactions from by-products available in large quantities at petroleum refineries have decided advantages in their favor for low cost production. 50

In the interest of improving compression-ignition fuels from all aspects, many organic compounds containing sulfur, nitrogen and oxygen have been tested and in accordance with this invention it has been found that organic com-

pounds containing an oxy-nitrogen sulfur group attached to carbon, are efficiently and economically useful in this object. The effectiveness of these compounds is surprisingly high compared with other nitrogen and sulfur containing compounds and accordingly is ascribed to the activity of their characteristic linkage, which may be graphically depicted as having some of the following structures and compositions: 5



These structures are capable of considerable modification and may be attached to a wide variety of organo radicals, but it is mainly essential that the oxy-nitrogen group be attached to carbon in an organic radical through a sulfur atom. 15

The following types of compounds containing active oxy-nitrogen sulfur groups may be used in accordance with the present invention: 20

Nitrosyl mercaptans or thionitrites having the general structural formulae: RSNO or



where R is an organo group such as an aliphatic or cyclic hydrocarbon radical, which may contain branched groups, e. g., ethyl nitrosyl mercaptan CH<sub>3</sub>SNO, isopropyl thionitrite (CH<sub>3</sub>)<sub>2</sub>CSNO, and triphenylmethyl thionitrite, (C<sub>6</sub>H<sub>5</sub>)<sub>3</sub>CSNO. 30

Sulphonium nitrates having the general structural formula:



where R stands for organo groups linked by three valence bonds to the sulfur, e. g., triethyl sulphonium nitrate (C<sub>2</sub>H<sub>5</sub>)<sub>3</sub>SNO<sub>3</sub>, and methyl diethyl sulphonium nitrate (C<sub>2</sub>H<sub>5</sub>)<sub>2</sub>CH<sub>3</sub>SNO<sub>3</sub>. 40

Sulfonyl hydroxyl amines are represented by RSO<sub>2</sub>NHOH in which R is an organo group, e. g., benzene sulfonyl hydroxyl amine.

Organic sulfur compounds, such as mercaptans and their derivatives, recovered in abundance in desulphurizing petroleum oils are by-products which have fuel value but which have been in general worthless for use in fuels on account of their offensive odor and the acidic nature of their combustion products. The mercaptans are represented by the general formula RSH, R being a hydrocarbon radical, and their resemblance to alcohols makes them known as thio-alcohols. 45

Alkyl thionitrites, which form a preferred class of ignition-promoting agents in the present invention, 50

10

15

20

30

35

40

45

50

55

may be regarded as esters of nitrous acid and thioalcohols.

It has been found possible to change mercaptans easily by reaction with nitrosyl chloride, 5 NOCl, or its equivalents, such as alkyl nitrites or nitrous acid, into compounds having a general formula R—S—NO, in which R is a hydrocarbon radical, for example, an alkyl or an aryl radical. A specific example is the reaction of butyl mercaptan, C<sub>4</sub>H<sub>9</sub>SH, with nitrosyl chloride at about 10 —5° C. to —10° C. to form butyl nitrosyl mercaptan. When the reaction is substantially completed as indicated by a greenish color of thick layers, the product may be purified simply by 15 washing with a cold alkaline solution and cold water. The general reaction may be represented by RSH+NOCl→RSNO+HCl.

Although the mercaptan class of compounds recovered as by-products in petroleum refineries 20 includes numerous compounds having various hydrocarbon radicals attached to the —SH group, by specific procedures for extraction of the mercaptans, as for example by an alkaline wash, and fractionation of the steam distilled extract, the 25 various types of mercaptans can be separately concentrated. Specific fractions of mercaptans having certain alkyl groups, normal or branched, attached to the —SH radical, e. g., the butyl mercaptans, and closely related mercaptans can 30 thus be concentrated. Among the related mercaptans which may be used are ethyl, propyl, amyl, hexyl, heptyl, and octyl mercaptans including the iso, primary, secondary, and tertiary 35 isomers. In general, such mercaptans and related organic sulfur compounds, whether recovered in petroleum refining or prepared synthetically, are considered suitable for preparing the promoters in accordance with the present invention in so far as they permit the linking of an 40 oxy-nitrogen group to the sulfur atom, whether this be obtained by any of the well known methods, such as substitution, addition, reaction with an oxy acid of nitrogen, etc. For example, 45 double decomposition reactions of mercaptans and mercaptide with nitrites or nitric oxide in the following ways are contemplated:



where R and R' represent organic radicals and M represents a metal in a mercaptide. The latter type of reaction is particularly advantageous 55 if an active metal is present in the mercaptide, because both products may then be used together or singly as addition agents.

The organic oxy-nitrogen sulfur compounds 60 described may be added in concentrations ranging from a fraction of 1% up to the limit of solubility in the fuel, but preferably from .025 to 3% to a hydrocarbon oil of suitable range for use as fuel in compression-ignition engines of the 65 Diesel type. A gas oil boiling from 400° F. to 700° F., or 750° F. may be used. Under some circumstances, a more narrowly cut fraction such as one distilling from about 400° to 600° F. or from 500° to 700° F. may be used.

70 Among mercaptans used the tertiary alkyl mercaptans, and particularly tertiary butyl mercaptans, have been found to lead to the production of nitrosyl mercaptans which are most effective ignition-promoters in Diesel fuels.

75 The effectiveness of tertiary butyl nitrosyl mer-

captan is demonstrated by the following tabulated results:

| Percent tert.-butyl nitrosyl mercaptan in colombia gas oil | Cetane number | Cetane number increase |
|------------------------------------------------------------|---------------|------------------------|
| 0                                                          | 38            | 0                      |
| 0.25                                                       | 47            | 9                      |
| 0.50                                                       | 49            | 11                     |
| 0.50                                                       | 51            | 13                     |
| 1.0                                                        | 55            | 17                     |
| 2.0                                                        | 61            | 23                     |
| 3.0                                                        | 64            | 26                     |

In testing the efficiency of these promoters the "cetane number" is recommended as a good 15 standard of evaluation by the S. A. E. Volunteer Group for Compression-Ignition Fuel Research. This test is described in the S. A. E. Journal of June 1936, page 225, and consists in a performance comparison of the fuel to be tested with 20 blends of cetane and alphamethyl-naphthalene. The percent cetane in the blend with the alphamethyl-naphthalene to give the same ignition quality test performance as the fuel in question is taken as the cetane number of that fuel. Normal cetane serves as a standard of high ignition 25 quality in Diesel fuel rating analogously to the way iso-octane is used as a standard of high anti-knock in gasoline rating. Normal cetane has a very short ignition lag in a compression-ignition 30 engine, whereas alphamethyl-naphthalene on the contrary has a long lag associated with poor ignition quality, and for a blend of these two hydrocarbons the ignition quality in terms of ignition lag is nearly inversely proportional to the concentration of the cetane. The time which passes between the beginning of the fuel injection into the combustion chamber of the test engine and the point at which ignition of the fuel sets in is called the ignition lag which may be 35 expressed in degrees of crank angle or in time units.

The tabulated results on the effect of varying 40 small percentages of the nitrosyl mercaptan in a Diesel fuel evince the excellent effectiveness of these compounds in improving ignition quality of the Diesel fuel as expressed by cetane number. The cetane number increase is a measure of the reduction in time lag and detonation effected by the nitrosyl mercaptan in terms of the corresponding improvement made by such an increase in percent of normal cetane in a blend with alphamethyl-naphthalene.

The small quantities of organic sulfur oxy-nitrogen compounds added for a substantial improvement of the Diesel fuel do not increase the sulfur content of the treated fuel excessively. It is recognized that a high content of sulfur may be considered undesirable in the operation of 55 some engines.

Advantageously for storage purposes, the promoters of this invention have the creditable property of being resistant to hydrolysis by water, although they may need some protection against unnecessary exposure to air.

This invention makes commercially feasible the preparation of Diesel fuels giving satisfactory engine performance from crude oils, gas oils, and residual fuels having low pour points, low A. P. I. gravities, and high heat values, procured 70 from naphthene base, asphalt base, and mixed base crudes, since the addition in small quantities of the nitrosyl mercaptan ignition-promoters improves their ignition qualities to the extent that they perform satisfactorily particularly in 75

high speed Diesel engines. The burning qualities of gas oils from paraffine crudes are also enhanced by the nitrosyl mercaptans. Ordinarily, the hydrocarbon fuel with which the promoter is blended for use in Diesel type engines has a boiling range above that of gasoline.

Small quantities of this promoter may be used for adapting various mixtures of hydrocarbons for use as Diesel fuels, including recycle reflux 10 from a cracking operation, oils from destructive distillations of pyro-bituminous and asphaltic materials, non-paraffinic extracts, and mixtures of these with one another or with crude petroleum fractions. Other agents for enhancing 15 various qualities without detracting substantially from the ignition qualities of the fuel, such as oiliness agents, sludge dispersers, dyes, corrosion inhibitors, anti-oxidants, viscosity improvers, and pour point depressants may be admixed 20 with the fuel as desired in addition to the nitrosyl mercaptan. Also, other promoters may be admixed.

It is not intended that this invention be limited to the specific examples which are given merely for the sake of illustration. It is intended to claim all the novelty inherent in the invention as broadly as the prior art permits in the 5 appended claims.

We claim:

1. A fuel for compression-ignition engines of the Diesel type comprising essentially a hydrocarbon fuel with which is blended a minor proportion of a tertiary alkyl nitrosyl mercaptan. 10
2. A fuel for compression-ignition engines of the Diesel type comprising essentially a hydrocarbon fuel with which is blended a minor proportion of tertiary butyl nitrosyl mercaptan. 15
3. A fuel for compression-ignition engines of the Diesel type comprising essentially gas oil petroleum hydrocarbons and about 0.25 to 3% of tertiary butyl nitrosyl mercaptan. 20

EUGENE LIEBER.  
PHARIS MILLER.